



US009790608B2

(12) **United States Patent**  
**Sista et al.**

(10) **Patent No.:** **US 9,790,608 B2**  
(45) **Date of Patent:** **Oct. 17, 2017**

(54) **METHODS OF FORMING BORIDED DOWN HOLE TOOLS**

(71) Applicant: **Baker Hughes Incorporated**, Houston, TX (US)

(72) Inventors: **Vivekanand Sista**, The Woodlands, TX (US); **John H. Stevens**, The Woodlands, TX (US); **James L. Overstreet**, Tomball, TX (US)

(73) Assignee: **Baker Hughes Incorporated**, Houston, TX (US)

(\*) Notice: Subject to any disclaimer, the term of this patent is extended or adjusted under 35 U.S.C. 154(b) by 633 days.

(21) Appl. No.: **14/019,132**

(22) Filed: **Sep. 5, 2013**

(65) **Prior Publication Data**

US 2015/0060288 A1 Mar. 5, 2015

(51) **Int. Cl.**

**C25D 3/66** (2006.01)  
**C25D 5/02** (2006.01)  
**C25D 11/00** (2006.01)  
**C25D 9/04** (2006.01)  
**C25D 11/02** (2006.01)

(52) **U.S. Cl.**

CPC ..... **C25D 3/66** (2013.01); **C25D 5/02** (2013.01); **C25D 9/04** (2013.01); **C25D 11/028** (2013.01)

(58) **Field of Classification Search**

CPC ..... C23C 22/70; C25D 3/66; C25D 3/665  
USPC ..... 205/230; 148/241, 242

See application file for complete search history.

(56)

**References Cited**

U.S. PATENT DOCUMENTS

3,634,145 A 1/1972 Homan  
3,697,390 A \* 10/1972 McCawley et al. .... C25D 9/08  
205/148  
4,188,242 A 2/1980 Scales  
4,210,497 A 7/1980 Bennstedt et al.  
4,499,795 A 2/1985 Radtke  
4,664,722 A \* 5/1987 Clinkscales ..... C21D 1/72  
148/212  
4,934,467 A \* 6/1990 Langford, Jr. .... E21B 10/25  
175/371  
6,478,887 B1 \* 11/2002 Sue ..... C23C 8/08  
148/279  
2010/0018611 A1 1/2010 Timur et al.  
2010/0133805 A1 6/2010 Stevens et al.  
2010/0224498 A1 9/2010 Ürgen et al.

(Continued)

FOREIGN PATENT DOCUMENTS

RO 69862 A2 \* 6/1981  
SU 328214 A \* 11/1972

OTHER PUBLICATIONS

Abstract translation of RO 69862 of Spataru, published 1981.\*

(Continued)

*Primary Examiner* — Brian W Cohen

(74) *Attorney, Agent, or Firm* — TraskBritt

(57) **ABSTRACT**

A method of forming a down-hole tool comprises contacting at least a portion of at least one down-hole structure comprising at least one ceramic-metal composite material with a molten electrolyte comprising sodium tetraborate. Electrical current is applied to at least a portion of the at least one down-hole structure to form at least one borided down-hole structure comprising at least one metal boride material. Other methods of forming a down-hole tool, and a down-hole tool are also described.

**18 Claims, 3 Drawing Sheets**



(56)

**References Cited**

## U.S. PATENT DOCUMENTS

- 2011/0073217 A1\* 3/2011 Smith ..... C23C 8/08  
148/279  
2011/0132769 A1\* 6/2011 Hurst ..... C25D 3/56  
205/157  
2012/0018141 A1 1/2012 John  
2012/0298425 A1 11/2012 De Maindreville et al.  
2013/0056363 A1 3/2013 Timur et al.

## OTHER PUBLICATIONS

- Abstract translation of SU 328214 of Voroshnin, published 1971.\* Translated Abstract of Lyakhovich et al "Low Temperature Boronizing", Metallovedenie i Termicheskaya Obrabotka Metallov, 1974.\* Atik et al., The Effects of Conventional Heat Treatment and Boronizing on Abrasive Wear and Corrosion of SAE 1010, SAE 1040, D2 and 304 Steels, Tribology International, vol. 36, (2003), pp. 155-161. Erdemir et al., Ultra-Fast Boriding for Improved Energy Efficiency and Reduced Emissions in Materials Processing Industries. Final Report, Energy Systems Division, Argonne National Laboratory, (Aug. 2012), 57 pages. Kahvecioglu et al., Ultra-Fast Boriding of Nickel Aluminide, Thin Solid Films, vol. 520, (2011), pp. 1575-1581.

Kartal et al., The Growth of Single Fe2B Phase on Low Carbon Steel via Phase Homogenization in Electrochemical Boriding, Surface & Coatings Technology, vol. 206, (2011), pp. 2005-2011.

Oliveira et al., Evaluation of Hard Coatings Obtained on AISI D2 Steel by Thermo-Reactive Deposition Treatment, Surface & Coatings Technology, vol. 201, (2006), pp. 1880-1885.

Sen et al., An Approach to Kinetic Study of Borided Steels, Surface & Coatings Technology, vol. 191, (2005), pp. 274-285.

Sista et al., Electrochemical Boriding and Characterization of AISI D2 Tool Steel, Electrochemical Boriding and Characterization of AISI D2 Tool Steel, Thin Solid Films, vol. 520, (2011), pp. 1582-1588.

Sista et al., Evaluation of Electrochemical Boriding of Inconel 600, Surface & Coatings Technology, vol. 215, (2013), pp. 452-459.

Greco, A. et al; "Friction and wear behaviour of boron based surface treatment and nano-particle lubricant additives for wind turbine gearbox applications" Wear, 2011, p. 1754-1760.

International Search Report for International Application No. PCT/US14/54269 dated Dec. 16, 2014, 3 pages.

International Written Opinion for International Application No. PCT/US14/54269 dated Dec. 16, 2014, 11 pages.

International Preliminary Report on Patentability for International Application No. PCT/US14/54269 dated Mar. 8, 2016, 11 pages.

\* cited by examiner



FIG. 1



FIG. 2



FIG. 3

## 1

METHODS OF FORMING BORIDED DOWN  
HOLE TOOLS

## TECHNICAL FIELD

Embodiments of the disclosure relate generally to methods of forming borided down-hole tools, and to related down-hole tools. More particularly, embodiments of the disclosure relate to methods of forming borided down-hole tools using electrochemical boronizing and to related down-hole tools.

## BACKGROUND

Wellbores are formed in subterranean formations for various purposes including, for example, extraction of oil and gas from the subterranean formations and extraction of geothermal heat from the subterranean formations. Wellbores can exhibit extremely aggressive environments. For example, wellbores can exhibit abrasive surfaces, can be filled with corrosive chemicals (e.g., caustic drilling muds; well fluids, such as salt water, crude oil, carbon dioxide, and hydrogen sulfide; etc.), and can exhibit increasing high temperatures and pressures at progressively deeper “down-hole” locations.

The extremely aggressive environments of wellbores can rapidly degrade the materials of structures, tools, and assemblies used in various down-hole applications (e.g., drilling applications, conditioning applications, logging applications, measurement applications, monitoring applications, exploring applications, etc.). Such degradation limits operational efficiency of these structures, tools and assemblies, and results in undesirable repair and replacement costs. Accordingly, there is a continuing need for down-hole structures, tools, and assemblies having material characteristics capable of withstanding such extremely aggressive environments, as well as for methods of forming such down-hole structures, tools, and assemblies.

One approach toward forming down-hole structures, tools, and assemblies capable of withstanding such extremely aggressive environments of wellbores includes boronizing the down-hole structures, tools, and assemblies. Boronizing, also known as “boriding,” is a thermal diffusion process wherein boron atoms diffuse into and react with metals to form metal borides exhibiting relatively enhanced properties (e.g., thermal resistance, hardness, toughness, chemical resistance, abrasion resistance, corrosion resistance, reduction in friction coefficient, mechanical strength, etc.) as compared to the metals. Unfortunately, however, conventional methods of forming borided down-hole structures, tools, and assemblies can be cost-prohibitive and environmentally unfriendly. For example, conventional methods of forming borided down-hole structures, tools, and assemblies can be time consuming (e.g., powder pack boriding, gas boriding, and fluidized bed boriding processes requiring from about 8 hours to about 10 hours of processing time; plasma boriding processes requiring from about 15 hours to about 25 hours of processing time; molten salt boriding processes requiring from about 6 hours to about 8 hours of processing time; etc.), and can utilize and produce toxic chemicals that necessitate the use of separate and costly equipment and processes to mitigate health, safety, and environmental concerns.

It would, therefore, be desirable to have new methods, systems, and apparatuses for forming borided down-hole structures, tools, and assemblies that are simple, fast, cost-effective, and environmentally friendly as compared to con-

## 2

ventional methods, systems, and apparatuses for forming borided down-hole structures, tools, and assemblies. Such methods, systems, and apparatuses may facilitate increased adoption and use of borided structures, tools, and assemblies in down-hole applications.

## BRIEF SUMMARY

Embodiments described herein include methods of forming borided down-hole tools, and related down-hole tools. For example, in accordance with one embodiment described herein, a method of forming a borided down-hole tool comprises contacting at least a portion of at least one down-hole structure comprising at least one ceramic-metal composite material with a molten electrolyte comprising sodium tetraborate ( $Na_2B_4O_7$ ). Electrical current is applied to the at least a portion of the at least one down-hole structure to form at least one borided down-hole structure comprising at least one metal boride material.

In additional embodiments, a method of forming a borided down-hole tool comprises at least partially inserting at least one down-hole structure comprising at least one ceramic-metal composite material into a molten electrolyte comprising  $Na_2B_4O_7$  at a temperature of from about 550° C. to about 1400° C. Electrical current is applied to the at least one down-hole structure for a period of time within a range of from about one (1) minute to about 5 hours to convert at least a portion of the at least one ceramic-metal composite material into at least one metal boride material and form at least one borided down-hole structure. The at least one borided down-hole structure is secured to at least one other down-hole structure.

In yet additional embodiments, a down-hole tool comprises at least one borided structure formed by the method comprising contacting at least a portion of the at least one structure comprising at least one ceramic-metal composite material with a molten electrolyte comprising  $Na_2B_4O_7$ , and applying electrical current to the at least a portion of the at least one structure in contact with the molten electrolyte to diffuse boron into the at least one structure and form at least one metal boride material.

## BRIEF DESCRIPTION OF THE DRAWINGS

While the specification concludes with claims particularly pointing out and distinctly claiming that which is regarded as the invention, advantages of the invention can be more readily ascertained from the following detailed description when read in conjunction with the accompanying drawings in which:

FIG. 1 is a longitudinal schematic view of a borided down-hole assembly, formed in accordance with an embodiment of the disclosure;

FIG. 2 is a simplified cross-sectional view of an electrochemical cell for producing a borided down-hole structure, in accordance with embodiments of the disclosure; and

FIG. 3 is a simplified cross-sectional view of a borided down-hole structure, formed in accordance with an embodiment of the disclosure.

## DETAILED DESCRIPTION

Methods of forming borided down-hole structures, tools, and assemblies are described, as are related down-hole structures, tools, and assemblies. For example, in some embodiments, a method of forming a borided down-hole tool includes inserting at least one down-hole structure

formed of and including a metal material, and at least two anodes into a molten electrolyte contained within a crucible to form an electrochemical cell. The down-hole structure may serve as a cathode of the electrochemical cell. Electrical current is applied to the electrochemical cell to diffuse boron atoms from the molten electrolyte into the down-hole structure and form at least one borided down-hole structure formed of and including a metal boride material. The borided down-hole structure may, optionally, be kept in the molten electrolyte material in the absence of electrical current for a sufficient period of time to facilitate phase homogenization of the metal boride material. The borided down-hole structure may be secured to at least one other down-hole structure to form a borided down-hole tool. The borided down-hole tool may be secured to at least one other down-hole tool to form a borided down-hole assembly. The borided down-hole structures, tools, and assemblies of the disclosure may exhibit enhanced properties (e.g., enhanced mechanical strength, wear resistance, thermal resistance, chemical resistance, corrosion resistance, etc.) favorable to the use thereof in down-hole applications. The methods of the disclosure may enable the borided down-hole structures, tools, and assemblies to be formed in a simpler, faster, more cost-effective, and in a more environmentally friendly manner as compared to conventional methods.

The following description provides specific details, such as material types, material thicknesses, and processing conditions in order to provide a thorough description of embodiments of the disclosure. However, a person of ordinary skill in the art will understand that the embodiments of the disclosure may be practiced without employing these specific details. Indeed, the embodiments of the disclosure may be practiced in conjunction with conventional fabrication techniques employed in the industry. In addition, the description provided below does not form a complete process flow for manufacturing a structure, tool, or assembly. The structures described below do not form a complete tool or a complete assembly. Only those process acts and structures necessary to understand the embodiments of the disclosure are described in detail below. Additional acts to form the complete tool or the complete assembly from various structures may be performed by conventional fabrication techniques. The drawings accompanying the application are for illustrative purposes only, and are not drawn to scale. Additionally, elements common between figures may retain the same numerical designation.

Although some embodiments of the disclosure are depicted as being used and employed in particular down-hole assemblies and components thereof, persons of ordinary skill in the art will understand that the embodiments of the disclosure may be employed in any down-hole assembly (e.g., drilling assembly, conditioning assembly, logging assembly, measurement assembly, a monitoring assembly, etc.), drill bit, drill string, and/or component of any thereof where it is desirable to enhance at least one of the wear resistance, thermal resistance, and chemical resistance of the down-hole assembly, drill bit, drill string, and/or component of any thereof during and/or after the formation of a wellbore in a subterranean formation. By way of non-limiting example, embodiments of the disclosure may be employed in earth-boring rotary drill bits, fixed-cutter drill bits, roller cone drill bits, hybrid drill bits employing both fixed and rotatable cutting structures, core drill bits, eccentric drill bits, bicenter drill bits, expandable reamers, expandable stabilizers, fixed stabilizers, mills, and other components of a down-hole assembly or drill string as known in the art.

As used herein, the singular forms "a," "an," and "the" are intended to include the plural forms as well, unless the context clearly indicates otherwise.

As used herein, the term "and/or" includes any and all combinations of one or more of the associated listed items.

As used herein, the term "substantially," in reference to a given parameter, property, or condition, means to a degree that one of ordinary skill in the art would understand that the given parameter, property, or condition is met with a small degree of variance, such as within acceptable manufacturing tolerances.

FIG. 1 is a longitudinal schematic representation of a borided down-hole assembly 100 for use during and/or after the formation of a wellbore 102 within a subterranean formation 104. As shown in FIG. 1, the borided down-hole assembly 100 may be provided into the wellbore 102. The borided down-hole assembly 100 may include at least one borided down-hole tool 108 formed in accordance with methods described hereinbelow. The borided down-hole tool 108 may include at least one borided structure or component, such as at least one borided external structure 106, and/or at least one borided internal structure 110. If present, the borided external structure 106 may at least partially surround (e.g., contain, hold, shield, etc.) at least one other structure or component of the borided down-hole tool 108, such as the borided internal structure 110. In turn, if present, the borided internal structure 110 may be at least partially surrounded (e.g., contained, held, shielded, etc.) by at least one other structure or component of the borided down-hole tool 108, such as the borided external structure 106. In some embodiments, the borided down-hole tool 108 comprises an earth-boring rotary drill bit including one or more of at least one borided internal surface (e.g., a borided bearing surface), and at least one borided external surface (e.g., a borided bit body surface, such as a borided bit blade surface).

An embodiment of the disclosure will now be described with reference to FIG. 2, which illustrates a simplified cross-sectional view of a configuration that may be used in a method of forming a borided down-hole structure (e.g., at least one borided structure of the borided down-hole tool 108 previously described with reference to FIG. 1, such as at least one of the borided external structure 106, and the borided internal structure 110) for a down-hole tool and/or assembly, in accordance with embodiments of the disclosure. The method includes providing a molten electrolyte 206, at least one down-hole structure 202, and at least two anodes 212 into a crucible 204 to form an electrochemical cell 200. Electrical current is then applied to the electrochemical cell 200 to boronize the down-hole structure 202. With the description as provided below, it will be readily apparent to one of ordinary skill in the art that the method described herein may be used in various applications. In other words, the method may be used whenever it is desired to form a borided structure for a down-hole application (e.g., a drilling application, a conditioning application, a logging application, a measurement application, a monitoring application).

The crucible 204 may be any vessel or container configured and of a material suitable for holding the molten electrolyte 206 before, during, and after the electrochemical boriding process of the disclosure, as described in further detail below. By way of non-limiting example, the crucible 204 may comprise a silicon carbide (SiC) crucible configured to receive and hold the molten electrolyte 206, the down-hole structure 202, and the at least two anodes 212. In additional embodiments, the crucible 204 may be formed of

and include nitride bonded SiC bricks. In further embodiments, the crucible 204 may be formed of and include an electrically conductive material that may serve as an anode during the electrochemical boronizing process. For example, the crucible 204 may be formed of and include a graphite material. The crucible 204 may be operatively associated with (e.g., connected to) at least one heating device (e.g., combustion heater, electrical resistance heater, inductive heater, electromagnetic heater, etc.) configured and operated to achieve and/or maintain a desired temperature of the molten electrolyte 206.

The molten electrolyte 206 may comprise at least one boron-containing material formulated for depositing boron (B) atoms onto and within the down-hole structure 202 during the electrochemical boronizing process, as described in further detail below. For example, the molten electrolyte 206 may comprise at least one of sodium tetraborate ( $Na_2B_4O_7$ ) (often referred to as “borax”), potassium borofluoride ( $KBF_4$ ), a boric acid, a boron oxide, and a borate of an element of Group 1 (e.g., lithium, sodium, potassium) or Group 2 (e.g., beryllium, magnesium, calcium, strontium, barium) of the Periodic Table of Elements. In some embodiments, the molten electrolyte 206 comprises about 100 percent by weight (wt %) molten anhydrous  $Na_2B_4O_7$ . In additional embodiments, the molten electrolyte 206 comprises a molten mixture of a boron-containing material (e.g.,  $Na_2B_4O_7$ ) and at least one other material, such as at least one of sodium fluoride ( $NaF$ ), sodium chloride ( $NaCl$ ), sodium hydroxide ( $NaOH$ ), sodium carbonate ( $Na_2CO_3$ ), sodium sulfite ( $Na_2SO_3$ ), sodium phosphate ( $Na_3PO_4$ ), calcium chloride ( $CaCl_2$ ), lithium chloride ( $LiCl$ ), barium chloride ( $BaCl_2$ ), and lead oxide ( $PbO$ ). The at least one other material may, for example, comprise from about 0 wt % to about 50 wt % of the molten electrolyte 206, with the at least one boron-containing material comprising a remainder of the molten electrolyte 206. By way of non-limiting example, the molten electrolyte 206 may comprise from about 50 wt % to about 90 wt % of the at least one boron-containing material, and from about 10 wt % to about 50 wt % of the at least one other material. In some embodiments, the molten electrolyte 206 comprises from about 50 wt % to about 90 wt %  $Na_2B_4O_7$ , and from about 10 wt % to about 50 wt % of at least one of  $Na_2SO_3$ ,  $NaOH$ ,  $Na_3PO_4$ , and  $PbO$ .

A temperature of the molten electrolyte 206 may be within a range of from about 550° C. to about 1400° C. The temperature of the molten electrolyte 206 may at least partially depend on the material composition of the molten electrolyte 206. The temperature of the molten electrolyte 206 may be at or above a melting point temperature of a solid precursor to the molten electrolyte 206. As a non-limiting example, in embodiments where the molten electrolyte 206 comprises a boron-containing material (e.g., from about 50 wt % to about 90 wt %  $Na_2B_4O_7$ ) and at least one other component (e.g., from about 10 wt % to about 50 wt % of at least one of  $Na_2SO_3$ ,  $NaOH$ ,  $Na_3PO_4$ ,  $PbO$ , etc.), the temperature of the molten electrolyte 206 may be within a range of from about 550° C. to about 700° C. As another non-limiting example, in embodiments where the molten electrolyte 206 comprises about 100 wt % of the boron-containing material (e.g., about 100 wt %  $Na_2B_4O_7$ ), the temperature of the molten electrolyte 206 may be within a range of from about 770° C. to about 1400° C., such as from about 850° C. to about 1200° C., from about 900° C. to about 1100° C., or from about 950° C. to about 1000° C. In some embodiments, the molten electrolyte 206 comprises 100 wt %  $Na_2B_4O_7$ , and the temperature of the molten electrolyte 206 is within a range of from about 950° C. to about 1000°

C. The molten electrolyte 206 may be formed within the crucible 204 (e.g., by heating the crucible 204 at least to the melting point of a solid precursor to the molten electrolyte 206), or may be formed outside the crucible 204 and then delivered into the crucible 204.

The anodes 212 may independently be formed of and include an electrically conductive material capable of withstanding the conditions (e.g., temperatures, materials, etc.) within the crucible 204. By way of non-limiting example, 10 each of the anodes 212 may be formed of and include graphite. In embodiments where the crucible 204 is configured to serve as an anode (e.g., where the crucible 204 is formed of and includes graphite), one or more of the anodes 212 may, optionally, be omitted. While various embodiments herein describe or illustrate the electrochemical cell 200 as including two anodes 212 the electrochemical cell 200 may, alternatively, include a different number of anodes 212. The number of anodes 212 provided into the molten electrolyte 206 may at least partially depend on the number 15 of down-hole structures 202 provided within the molten electrolyte 206. As a non-limiting example, if more than one down-hole structure 202 is provided into the molten electrolyte 206, more than two anodes 212 may also be provided into the molten electrolyte 206.

As depicted in FIG. 2, the anodes 212 may be electrically connected (e.g., directly connected, or indirectly connected) 25 to fixtures 210 configured (e.g., sized and shaped) to position, and hold or contain the anodes 212 within the crucible 204. The anodes 212 may be integral with their respective fixtures 210 (i.e., at least one of the anodes 212 and at least one of the fixtures 210 may comprise a single structure), or 30 may be discrete from their respective fixtures 210 (i.e., at least one of the anodes 212 and at least one of the fixtures 210 may comprise different, connected structures). If the anodes 212 and their respective fixtures 210 are discrete 35 structures, the fixtures 210 and the anodes 212 may be formed of and include the same material, or may be formed of and include different materials (e.g., different electrically conductive materials). In addition, if discrete structures, the anodes 212 and their respective fixtures 210 may be coupled to one another through conventional means which are not 40 described in detail herein.

The down-hole structure 202 may comprise any structure 45 associated with a down-hole tool and/or assembly. Accordingly, the down-hole structure 202 may exhibit a desired shape (i.e., geometric configuration) and size, such as a shape and size associated with a conventional structure or component of a down-hole tool. For example, the down-hole structure 202 may exhibit a conical shape, tubular shape, a 50 pyramidal shape, a cubical shape, cuboidal shape, a spherical shape, a hemispherical shape, a cylindrical shape, a semicylindrical shape, truncated versions thereof, or an irregular shape. Irregular shapes include complex shapes, 55 such as shapes associated with down-hole tools and/or assemblies. In some embodiments, the down-hole structure 202 exhibits the shape of a structure (e.g., an internal structure, such as a bearing; or an external structure, such as a blade, wear insert, cutting element, roller cone, roller cone insert, etc.) of a earth-boring rotary drill bit (e.g., a fixed-cutter drill bit, a roller cone drill bit, a hybrid drill bit employing both fixed and rotatable cutting structures, a core 60 drill bit, an eccentric drill bit, a bicenter drill bit, etc.), a completion tool (e.g., a packer, a screen, a bridge plug, a latch, a shoe, a nipple, a barrier, a sleeve, a valve, a pump, etc.), an expandable reamer, an expandable stabilizer, a fixed stabilizer, a slip-on stabilizer, a clamped-on stabilizer, an integral stabilizer, an ONTRAK™ tool, an optimized rota-

tional density tool, an AZIONTRAK™ tool, a slimhole neutron density tool, a calibrated neutron density tool, a drill motor, a bearing, an upper bearing housing, a lower bearing housings, a mud motor, a rotor, a stator, a pump, or a valve.

As depicted in FIG. 2, the down-hole structure 202 may be electrically connected (e.g., directly connected, or indirectly connected) to at least one fixture 214 configured (e.g., sized and shaped) to position, and hold or contain the down-hole structure 202 within the crucible 204. The fixture 214 be formed of and include an electrically conductive material capable of withstanding the conditions (e.g., temperature, materials, etc.) within the crucible 204. The down-hole structure 202 may be integral with the fixture 214 (i.e., down-hole structure 202 and the fixture 214 may comprise a single structure), or may be discrete from the fixture 214 (i.e., the down-hole structure 202 and the fixture 214 may comprise different, connected structures). If the down-hole structure 202 and the fixture 214 are discrete structures, the fixture 214 and the down-hole structure 202 may be formed of and include the same material, or may be formed of and include different materials (e.g., different electrically conductive materials). In addition, if discrete structures, the down-hole structure 202 and the fixture 214 and may be coupled to one another through conventional means which are not described in detail herein.

While various embodiments herein describe or illustrate a single down-hole structure 202 within the crucible 204, multiple down-hole structures may be provided within the crucible 204. The multiple down-hole structures may be held by a single fixture (e.g., the fixture 214) within the crucible 204, or may be held by multiple fixtures within the crucible 204. Each of the down-hole structures may be substantially the same, or at least one of the down-hole structures may be different than at least one other of the down-hole structures. Providing multiple down-hole structures within the crucible 204 may facilitate the simultaneous formation of multiple down-hole tools and/or assemblies. By way of non-limiting example, the crucible 204 may be at least partially filled with a plurality of down-hole structures such that at least a portion of each of the down-hole structures (e.g., the down-hole structure 202) is borided during subsequent electrochemical boronizing processing.

The down-hole structure 202 may be at least partially formed of (e.g., a laminate or other composite structure) and include a metal material capable of forming a hard, wear resistant (e.g., abrasion resistant, erosion resistant), and chemically resistant (e.g., corrosion resistant) metal boride material when subjected to the electrochemical boronizing process of the disclosure. The down-hole structure 202 may, for example, be at least partially formed of and include iron (Fe), cobalt (Co), nickel (Ni), copper (Cu), tungsten (W), titanium (Ti), molybdenum (Mo), niobium (Nb), vanadium (V), hafnium (Hf), tantalum (Ta), chromium (Cr), zirconium (Zr), aluminum (Al), silicon (Si), carbides thereof, nitrides thereof, oxides thereof, alloys thereof, or combinations thereof. The down-hole structure 202 may serve as a cathode of the electrochemical cell 200.

As a non-limiting example, the down-hole structure 202 may be formed of and include a metal alloy, such as at least one of an Fe-containing alloy, a Ni-containing alloy, a Co-containing alloy, an Fe- and Ni-containing alloy, a Co- and Ni-containing alloy, an Fe- and Co-containing alloy, an Al-containing alloy, a Cu-containing alloy, a Mg-containing alloy, and a Ti-containing alloy. In some embodiments, the down-hole structure 202 is formed of and includes a Fe-containing alloy (e.g., a steel-alloy). Suitable Fe-containing alloys are commercially available from numerous sources,

such as from Special Metals Corp., of New Hartford, N.Y., under the trade name INCONEL® (e.g., INCONEL® 945, INCONEL® 925, INCONEL® 745, INCONEL® 718, INCONEL® 600, etc.), and from Schoeller Bleckmann Sales Co. of Houston, Tex. (e.g., P550 alloy steel, P650 alloy steel, P750 alloy steel, etc.). The down-hole structure 202 may, for example, be formed of and include at least one of AISI 4815 alloy steel, AISI 4130M7 alloy steel, AISI 4140 alloy steel, AISI 4145H alloy steel, AISI 4715 alloy steel, AISI 8620 alloy steel, AISI 8630 alloy steel, SAE PS55 alloy steel, P550 alloy steel, P650 alloy steel, P750 alloy steel, INCONEL® 945, INCONEL® 925, and INCONEL® 745. In some embodiments, the down-hole structure 202 is formed of and includes at least one of AISI 4815 alloy steel, and AISI 4140 alloy steel.

As an additional non-limiting example, the down-hole structure 202 may be formed of and include a ceramic-metal composite material (i.e., a “cermet” material). The ceramic-metal composite material may include hard ceramic phase particles (or regions) dispersed throughout a matrix of metal material. The hard ceramic phase particles may comprise carbides, nitrides, and/or oxides, such as carbides of at least one of W, Ti, Mo, Nb, V, Hf, Ta, Cr, Zr, Al, and Si. For example, the hard ceramic phase particles may comprise one or more of tungsten carbide (WC), fused tungsten carbide (WC/W<sub>2</sub>C eutectic), titanium carbide (TiC), tantalum carbide (TaC), chromium carbide (CrC), titanium nitride (TiN), aluminum oxide (Al<sub>2</sub>O<sub>3</sub>), aluminum nitride (AlN), and silicon carbide (SiC). The hard ceramic phase particles may be substantially free of anomalies (e.g., attached materials, structures, etc.) that may otherwise impede or even prevent desired boronization of the hard ceramic phase particles. The hard ceramic phase particles may be monodisperse, wherein all of the hard ceramic phase particles are of substantially the same size, or may be polydisperse, wherein the hard ceramic phase particles have a range of sizes and are averaged. The matrix of metal material may, for example, comprise at least one of an Fe-containing alloy, a Ni-containing alloy, a Co-containing alloy, an Fe- and Ni-containing alloy, a Co- and Ni-containing alloy, an Fe- and Co-containing alloy, an Al-containing alloy, a Cu-containing alloy, a Mg-containing alloy, and a Ti-containing alloy. The matrix of metal material may also be selected from commercially pure elements such as Ni, Fe, Co, Al, Cu, Mg, and Ti. In some embodiments, the down-hole structure 202 is formed of and includes a ceramic-metal composite material comprising WC particles dispersed throughout a matrix of Ni.

The down-hole structure 202 may be conditioned to improve one or more properties thereof (e.g., thermal resistance, hardness, toughness, chemical resistance, wear resistance, friction coefficient, mechanical strength, etc.) prior to performing the electrochemical boronizing process of the disclosure. By way of non-limiting example, at least a portion of the down-hole structure 202 may be subjected to a conventional carburization process prior to being provided into the molten electrolyte 206 within the crucible 204. The down-hole structure 202 may, for example, comprise an at least partially carburized metal material, such as an at least partially carburized metal (e.g., Fe, Ni, Co, W, Ti, Mo, Nb, V, Hf, Ta, Cr, Zr, Al, etc.), and/or an at least partially carburized metal alloy (e.g., an Fe-containing alloy, a Ni-containing alloy, a Co-containing alloy, an Fe- and Ni-containing alloy, a Co- and Ni-containing alloy, an Fe- and Co-containing alloy, an Al-containing alloy, a Cu-containing alloy, a Mg-containing alloy, a Ti-containing alloy, etc.). In some embodiments, the down-hole structure 202 comprises a carburized Fe-containing alloy (e.g., a carburized steel

alloy). In additional embodiments, the down-hole structure 202 comprises a carburized ceramic-metal composite material.

The down-hole structure 202 may be cleaned prior to performing the electrochemical boronizing process of the disclosure. For example, at least a portion of the down-hole structure 202 may be subjected to a conventional cleaning process (e.g., a conventional volatilization process) prior to being provided into the molten electrolyte 206 within the crucible 204. The cleaning process may remove anomalies (e.g., attached materials, structures, etc.) from one or more surface(s) of the down-hole structure 202 that may otherwise impede or even prevent desired boronization of the down-hole structure 202.

The down-hole structure 202 may have a substantially homogeneous distribution of the metal material, or may include a substantially heterogeneous distribution of the metal material. As used herein, the "homogeneous distribution" means that amounts of a material (e.g., the metal material) do not vary throughout different portions (e.g., different lateral and longitudinal portions) of a structure. For example, if the down-hole structure 202 includes a substantially homogeneous distribution of the metal material, amounts of the metal material may not vary throughout different portions of the down-hole structure 202. The down-hole structure 202 may, for example, comprise a bulk structure of the metal material. In contrast, as used herein, the term "heterogeneous distribution" means amounts of a material (e.g., a metal material) vary throughout different portions of a structure. Amounts of the material may vary stepwise (e.g., change abruptly), or may vary continuously (e.g., change progressively, such as linearly, parabolically, etc.) throughout different portions of the structure. For example, if the down-hole structure 202 includes a substantially heterogeneous distribution of the metal material, amounts of the metal material may vary throughout at least one of different lateral portions and different longitudinal portions of the down-hole structure 202. The down-hole structure 202 may, for example, include an at least partial coating of the metal material on another material. If the down-hole structure 202 is formed of or includes a ceramic-metal composite material, the down-hole structure 202 may have a substantially homogeneous distribution of the ceramic-metal composite material, or may have a substantially heterogeneous distribution of the ceramic-metal composite material. In addition, the ceramic-metal composite material may include a substantially homogeneous distribution of the hard ceramic phase particles, or may include a substantially heterogeneous distribution of the hard ceramic phase particles.

Regardless of whether the metal material (and/or the ceramic-metal composite material) is homogeneously distributed or heterogeneously distributed, the down-hole structure 202 may include at least one metal-containing surface 208. As used herein, the term "metal-containing surface" means and includes a surface at least partially formed of and including the metal material (e.g., Fe, Ni, W, Co, Cu, Ti, Mo, Nb, V, Hf, Ta, Cr, Zr, Si, alloys thereof, combinations thereof, etc.). The metal-containing surface 208 may, for example, comprise at least one of an Fe-containing surface, an Ni-containing surface, a Co-containing surface, and a W-containing surface. The metal-containing surface 208 may be substantially free of anomalies (e.g., attached materials, structures, etc.) that may otherwise impede or even prevent desired boronization of the metal-containing surface 208. The metal-containing surface may be converted to a metal boride-containing surface upon exposure to the elec-

trochemical boronizing process, as described in further detail below. As used herein, the term "metal boride-containing surface" means and includes a surface at least partially formed of and including the metal boride material (e.g., an Fe boride, such as FeB, and/or Fe<sub>2</sub>B; a Ni boride, such as NiB, Ni<sub>2</sub>B, Ni<sub>3</sub>B and/or Ni<sub>4</sub>B<sub>3</sub>; a W boride, such as WB, WB<sub>2</sub>, W<sub>2</sub>B<sub>5</sub>, and/or WB<sub>4</sub>; a Co boride, such as CoB, Co<sub>2</sub>B, and/or Co<sub>3</sub>B; a Cu boride; a Ti boride, such as TiB, and/or TiB<sub>2</sub>; a Mo boride, such as MoB, Mo<sub>2</sub>B, MoB<sub>2</sub>, Mo<sub>2</sub>B<sub>5</sub>, and/or MoB<sub>4</sub>; a Nb boride, such as NbB, and/or NbB<sub>2</sub>; a V boride, such as VB, VB<sub>2</sub>, and/or V<sub>2</sub>B<sub>5</sub>; a Hf boride, such as HfB<sub>2</sub>; a Ta boride, such as TaB<sub>2</sub>; a Cr boride, such as CrB, and/or Cr<sub>2</sub>B; a Zr boride, such as ZrB<sub>2</sub>; a Si boride; combinations thereof; etc.). In some embodiments, each surface of the down-hole structure 202 comprises a metal-containing surface. In additional embodiments, the down-hole structure 202 includes at least one metal-containing surface and at least one non-metal-containing surface. By way of non-limiting example, an outer surface of the down-hole structure 202 may comprise a metal-containing surface, and an inner surface of the down-hole structure 202 may comprise a non-metal-containing surface.

An entirety of the metal-containing surface 208 of the down-hole structure 202 may be exposed to the molten electrolyte 206, or less than an entirety of the metal-containing surface 208 of the down-hole structure 202 may be exposed to the molten electrolyte 206. For example, at least one portion of the metal-containing surface 208 of the down-hole structure 202 may be covered or masked to substantially limit or prevent the boronization thereof during the electrochemical boronizing process. As another example, only a portion of the metal-containing surface 208 of the down-hole structure 202 may be provided (e.g., immersed, submerged, soaked, etc.) in the molten electrolyte 206. In some embodiments, an entirety of the metal-containing surface 208 of the down-hole structure 202 is exposed to the molten electrolyte 206 in the crucible 204.

With continued reference to FIG. 2, electrical current may be applied to the electrochemical cell 200 to boronize the down-hole structure 202. By way of non-limiting example, in embodiments where the molten electrolyte 206 comprises 100 wt % molten Na<sub>2</sub>B<sub>4</sub>O<sub>7</sub>, the applied electrical current may facilitate the extraction and deposition of B atoms on at least the metal-containing surface 208 of the down-hole structure 202 through the following reactions:



In additional embodiments where the molten electrolyte 206 includes at least one other material (e.g., at least one of NaF, NaCl, NaOH, Na<sub>2</sub>CO<sub>3</sub>, Na<sub>3</sub>PO<sub>4</sub>, Na<sub>2</sub>SO<sub>3</sub>, CaCl<sub>2</sub>, LiCl, BaCl<sub>2</sub>, and PbO), the other material may enhance or accelerate the extraction and deposition of B atoms from the boron-containing material (e.g., Na<sub>2</sub>B<sub>4</sub>O<sub>7</sub>, KBF<sub>4</sub>, a boric acid, a boron oxide, a borate of an element of Group 1 or Group 2 of the Periodic Table of Elements, etc.). The boron atoms may infiltrate or permeate the down-hole structure

## 11

202, and may react with at least a portion of the metal material thereof to form a boronized down-hole structure 202' including at least one metal boride material 216, as depicted in FIG. 3. As a non-limiting example, if the down-hole structure 202 is formed of and includes an Fe-containing alloy (e.g., a steel alloy, such as AISI 4815 alloy steel, AISI 4130M7 alloy steel, AISI 4140 alloy steel, AISI 4145H alloy steel, AISI 4715 alloy steel, AISI 8620 alloy steel, AISI 8630 alloy steel, SAE PS55 alloy steel, P550 alloy steel, P650 alloy steel, P750 alloy steel, INC-ONEL® 945, INCONEL® 925, INCONEL® 745, etc.), the liberated B atoms may diffuse into the down-hole structure 202 (FIG. 2) and react with the Fe atoms thereof to form a metal boride material 216 comprising at least one Fe boride phase through the following reactions:



As another non-limiting example, if the down-hole structure 202 is formed of and includes a ceramic-metal composite material (e.g., WC particles in a matrix of a metal material, such as a matrix of Ni), the liberated B atoms may diffuse into the down-hole structure 202 (FIG. 2) and react with the metal atoms of least one of the hard ceramic phase particles and the matrix of metal material to form a metal boride material 216 comprising hard ceramic phase particles in a matrix of at least one metal boride (e.g., WC particles in a matrix of at least one of a Ni boride and a W boride).

The metal boride material 216 may comprise a single layer of material, or may comprise multiple layers of material. If the metal boride material 216 comprises a single layer of material, the single layer of material may comprise multiple metal boride phases (e.g.,  $\text{Fe}_2\text{B}$  and  $\text{FeB}$ ), or may comprise a single metal boride phase (e.g.,  $\text{Fe}_2\text{B}$  or  $\text{FeB}$ ). In addition, if the metal boride material 216 comprises a multiple layers of material, at least one of the layers may include a different amount of at least one metal boride phase (e.g.,  $\text{Fe}_2\text{B}$  or  $\text{FeB}$ ) than at least one other of the layers. The metal boride material 216 may also comprise multiple metal borides. For example, if the down-hole structure 202 is formed of and includes an Fe-containing alloy including Cr, the metal boride material 216 may comprise at least one Fe boride (e.g.,  $\text{Fe}_2\text{B}$  and/or  $\text{FeB}$ ) and at least one Cr boride (e.g.,  $\text{Cr}_2\text{B}$  and/or  $\text{CrB}$ ). As another example, if the down-hole structure 202 is formed of and includes a ceramic-metal composite material including WC particles dispersed in a matrix of Ni, the metal boride material 216 may comprise WC particles within a matrix of at least one Ni boride and at least one W boride.

With reference to FIG. 3, electrical current may be applied to the electrochemical cell 200 (FIG. 2) for a sufficient period of time to form the metal boride material 216 to a desired thickness  $T_1$ , such as a thickness  $T_1$  within a range of from about 5 micrometers ( $\mu\text{m}$ ) to about 400 micrometers ( $\mu\text{m}$ ). The duration of the applied electrical current, and the resulting thickness  $T_1$  and material composition of the metal boride material 216 may at least partially depend on the material composition of the down-hole structure 202 (FIG. 2), the material composition and temperature of the molten electrolyte 206 (FIG. 2), and the applied current density. By way of non-limiting example, the applied current density may be within a range of from about 50 milliamperes per square centimeter ( $\text{mA}/\text{cm}^2$ ) to about 700  $\text{mA}/\text{cm}^2$  (e.g., from about 100  $\text{mA}/\text{cm}^2$  to about 500  $\text{mA}/\text{cm}^2$ , from about 100  $\text{mA}/\text{cm}^2$  to about 300  $\text{mA}/\text{cm}^2$ , or from about 100  $\text{mA}/\text{cm}^2$  to about 200  $\text{mA}/\text{cm}^2$ ), and the duration of the

## 12

applied electrical current may be within a range of from about 1 minute to about 5 hours (e.g., from about 1 minute to about 2 hours, or from about 1 minute to about 1 hour). In some embodiments, the current density is within a range of from about 100  $\text{mA}/\text{cm}^2$  to about 200  $\text{mA}/\text{cm}^2$ , and the duration of the applied electrical current is within a range of from about 1 minute to about 2 hours.

Following the formation of the metal boride material 216, the applied electrical current may be discontinued, and the borided down-hole structure 202' may, optionally, be kept in the molten electrolyte 206 (FIG. 2) for an additional period of time. Keeping the borided down-hole structure 202' in the molten electrolyte 206 in the absence of the applied electrical current (i.e., without any polarization) may facilitate phase homogenization in the metal boride material 216. By way of non-limiting example, in embodiments where the metal boride material 216 comprises an  $\text{Fe}_2\text{B}$  phase and an  $\text{FeB}$  phase (e.g., in a single layer, in separate layers, or a combination thereof), keeping the borided down-hole structure 202' in the molten electrolyte 206 for an additional period of time may enable at least a portion of the  $\text{FeB}$  phase of the metal boride material 216 to be converted to the  $\text{Fe}_2\text{B}$  phase. As compared the  $\text{FeB}$  phase, the  $\text{Fe}_2\text{B}$  phase may exhibit properties (e.g., improved toughness, improved hardness, etc.) favorable to the use of the borided down-hole structure 202' in down-hole applications. In some embodiments, substantially all of the  $\text{FeB}$  phase may be converted to the  $\text{Fe}_2\text{B}$  phase. As a non-limiting example, after discontinuing the applied electrical current, the borided down-hole structure 202' may be kept in the molten electrolyte 206 for a period of time with a range of from about 10 minutes to about two (2) hours (e.g., from about 15 minutes to about 45 minutes, or from about 15 minutes to about 30 minutes). In additional embodiments, the borided down-hole structure 202' may be removed from the molten electrolyte 206 without keeping the borided down-hole structure 202' in the molten electrolyte 206 for the additional period of time (i.e., without keeping the borided down-hole structure 202 in the molten electrolyte 206 for a period of time greater than or equal to about 10 minutes). In further embodiments, the borided down-hole structure 202' may be removed from the molten electrolyte 206 without keeping the borided down-hole structure 202' in the molten electrolyte 206 for the additional period of time, and may be provided into a different device or apparatus (e.g., a high temperature furnace) configured and operated to facilitate phase homogenization in the metal boride material 216.

The borided down-hole structure 202' may be removed from the crucible 204 (and the fixture 214), and may, optionally, be subjected to additional processing or conditioning. Additional processing may, for example, be utilized to enhance one or more properties of the borided down-hole structure 202' (e.g., thermal resistance, hardness, toughness, chemical resistance, corrosion resistance, wear resistance, lower friction coefficient, mechanical strength, etc.). By way of non-limiting example, at least a portion of the borided down-hole structure 202' may be subjected to a conventional carburization process. For example, borided portions of the borided down-hole structure 202' may be covered or masked, and at least one non-borided portion of the borided down-hole structure 202' may be conventionally carburized. The additional processing may also be utilized to prepare (e.g., shape, size, condition, etc.) the borided down-hole structure 202' to be secured to at least one other structure to form a desired down-hole tool (e.g., an earth-boring rotary drill bit, an expandable reamer, an expandable stabilizer, a fixed stabilizer, a rotor, a stator, a pump, a valve, etc.).

Following formation (and, optionally, additional processing), the borided down-hole structure 202' may be secured to (e.g., directly or indirectly attached to, provided within, etc.) at least one other structure to form a desired borided down-hole tool (e.g., the borided down-hole tool 108 previously described in relation to FIG. 1). The other structure may be substantially the same as the borided down-hole structure 202' (e.g., may exhibit substantially the same shape, size, and material configuration as the borided down-hole structure 202'), or may be different than the borided down-hole structure 202' (e.g., may exhibit at least one of a different shape, a different size, and a different material configuration than the borided down-hole structure 202'). For example, the other structure may comprise another borided down-hole structure, or may comprise a non-borided down-hole structure (i.e., a structure substantially free of at least one metal boride material). If the other structure comprises another borided down-hole structure, the other structure may have substantially the same shape, size, and material configuration as the borided down-hole structure 202', or may have at least one of a different shape, different size, and different material configuration than the borided down-hole structure 202'. In some embodiments, the other structure exhibits a different thickness of a metal boride material than the borided down-hole structure 202'.

The borided down-hole tool (e.g., the borided down-hole tool 108 previously described in relation to FIG. 1) including the borided down-hole structure 202' may be secured (i.e., directly secured, or indirectly secured) to at least one other down-hole tool to form a borided down-hole assembly (e.g., the borided down-hole assembly 100 previously described in relation to FIG. 1). The other down-hole tool may comprise another borided down-hole tool, or may comprise a non-borided down-hole tool. If the other down-hole tool comprises another borided down-hole tool, the other down-hole tool may have substantially the same shape, size, and material configuration as the borided down-hole tool, or may have at least one of a different shape, a different size, and a different material configuration than the borided down-hole tool. In some embodiments, the other down-hole tool exhibits a different thickness of a metal boride material than the borided down-hole tool.

The methods of the disclosure facilitate the fast, simple, cost-effective, and environmentally friendly formation of borided down-hole structures, tools, and assemblies able to withstand the aggressive environmental conditions (e.g., abrasive materials, corrosive chemicals, high temperatures, high pressures, etc.) frequently experienced in down-hole applications (e.g., drilling applications, conditioning applications, logging applications, measurement applications, monitoring applications, etc.). The borided down-hole structures, tools, and assemblies formed by the methods of the disclosure may also exhibit improved properties (e.g., metal boride material thickness and homogeneity, hardness, toughness, chemical resistance, etc.) as compared to borided down-hole structures formed by many conventional boronizing processes. As a result, the methods of the disclosure may be used to form borided down-hole structures, tools, and assemblies more rapidly and uniformly, improving production efficiency and increasing the quality and longevity of the down-hole structures, tools, and assemblies produced.

While the disclosure has been described herein with respect to certain embodiments, those of ordinary skill in the art will recognize and appreciate that it is not so limited. Rather, many additions, deletions and modifications to the embodiments described herein may be made without depart-

ing from the scope of the invention as hereinafter claimed. In addition, features from one embodiment may be combined with features of another embodiment while still being encompassed within the scope of the invention as contemplated by the inventor.

What is claimed is:

1. A method of forming a down-hole tool, comprising: directly contacting a surface of a ceramic-metal composite material of a down-hole structure with a molten electrolyte comprising  $\text{Na}_2\text{B}_4\text{O}_7$  and  $\text{PbO}$ , wherein the molten electrolyte comprises from about 50 wt % to about 90 wt % of  $\text{Na}_2\text{B}_4\text{O}_7$  and from about 10 wt % to about 50 wt %  $\text{PbO}$ , the ceramic-metal composite material of the down-hole structure comprising hard ceramic phase particles in a meta material matrix; and applying electrical current to the down-hole structure to convert at least a portion of the metal material matrix of the ceramic-metal composite material into a metal boride matrix and provide the ceramic-metal composite material with a metal boride-containing surface.

2. The method of claim 1, wherein directly contacting a surface of a ceramic-metal composite material of a down-hole structure further comprises selecting the down-hole structure to comprise a component of an earth-boring rotary drill bit, a completion tool, an expandable reamer, an expandable stabilizer, a fixed stabilizer, a slip-on stabilizer, a clamped-on stabilizer, an integral stabilizer, an optimized rotational density tool, a slimhole neutron density tool, a calibrated neutron density tool, a drill motor, a bearing, an upper bearing housing, a lower bearing housing, a rotor, a stator, a pump, or a valve.

3. The method of claim 1, further comprising selecting the ceramic-metal composite material to comprise tungsten carbide particles in a matrix of nickel.

4. The method of claim 1, further comprising maintaining a temperature of the molten electrolyte within a range of from about 550° C. to about 700° C.

5. The method of claim 1, wherein directly contacting a surface of a ceramic-metal composite material of a down-hole structure with a molten electrolyte comprises directly contacting only a portion of the surface of the ceramic-metal composite material with the molten electrolyte.

6. The method of claim 1, wherein applying electrical current to the down-hole structure comprises applying a current density within a range of from about 100 mA/cm<sup>2</sup> to about 700 mA/cm<sup>2</sup> for a period of time within a range of from about one (1) minute to about five (5) hours.

7. The method of claim 1, further comprising soaking the down-hole structure in the molten electrolyte in the absence of the electrical current after the application thereof to increase the phase homogeneity of at least a portion of the ceramic-metal composite material.

8. The method of claim 7, wherein soaking the down-hole structure in the molten electrolyte in the absence of the electrical current after the application thereof comprises at least partially immersing the down-hole structure in the molten electrolyte for a period of time within a range of from about one (1) minute to about one (1) hour.

9. A method of forming a down-hole tool, comprising: at least partially inserting at least one down-hole structure having a surface comprising hard ceramic phase particles in a metal matrix into a molten electrolyte consisting of anhydrous  $\text{Na}_2\text{B}_4\text{O}_7$  at a temperature of from about 770° C. to about 1400° C.; applying electrical current to the at least one down-hole structure for a period of time within a range of from about one (1) minute to about five (5) hours to convert

## 15

at least a portion of the metal matrix into a metal boride matrix and form at least one borided down-hole structure; masking the ceramic-metal composite material; carburizing at least one non-borided portion of the at least one borided down-hole structure after masking the ceramic-metal composite material; and securing the at least one borided down-hole structure to at least one other down-hole structure.

10. The method of claim 9, wherein securing the at least one borided down-hole structure to at least one other down-hole structure comprises securing the at least one borided down-hole structure to at least one other borided down-hole structure.

11. The method of claim 10, wherein securing the at least one borided down-hole structure to at least one other down-hole structure comprises securing the at least one borided down-hole structure to at least one structure exhibiting a different thickness of metal boride matrix than the at least one borided down-hole structure.

12. The method of claim 9, wherein securing the at least one borided down-hole structure to at least one other down-hole structure comprises coupling the at least one borided down-hole structure with the at least one other down-hole structure to form at least one of an earth-boring rotary drill bit, an expandable reamer, an expandable stabilizer, a fixed stabilizer, a rotor, a stator, a pump, and a valve.

## 16

13. The method of claim 1, wherein applying electrical current to the down-hole structure further comprises boronizing the hard ceramic phase particles of the ceramic-metal composite material.

14. The method of claim 13, wherein boronizing the hard ceramic phase particles of the ceramic-metal composite material comprises reacting metal atoms of the hard ceramic phase particles with boron liberated from the  $\text{Na}_2\text{B}_4\text{O}_7$  during the application of the electrical current.

15. The method of claim 1, further comprising selecting the ceramic-metal composite material to exhibit a substantially homogeneous distribution of the hard ceramic phase particles in the metal matrix material.

16. The method of claim 1, wherein directly contacting a surface of a ceramic-metal composite material of a down-hole structure with a molten electrolyte comprises selecting the molten electrolyte to consist of  $\text{Na}_2\text{B}_4\text{O}_7$  and  $\text{PbO}$ .

17. The method of claim 1, further comprising selecting the down-hole structure to comprise a layer of the ceramic-metal composite material only partially covering another material.

18. The method of claim 1, further comprising: masking the ceramic-metal composite material; and carburizing at least one non-borided portion of the borided down-hole structure after masking the ceramic-metal composite material.

\* \* \* \* \*